

## UNITED STATES PATENT OFFICE

1,972,092

## CELLULOSE DERIVATIVE COMPOSITION

George De Witt Graves and Walter Eastby  
Lawson, Wilmington, Del., assignors to E. I.  
du Pont de Nemours & Company, Wilmington,  
Del., a corporation of Delaware

No Drawing. Application December 8, 1932,  
Serial No. 646,298

16 Claims. (Cl. 106—37)

This invention relates to cellulose derivative compositions, and more particularly, to such compositions including as plasticizers therefor organic polycarboxylic acid esters containing an esterified higher alkyl group. This application is a continuation in part of Graves and Lawson United States application Serial No. 543,387, filed June 10, 1931, entitled "Cellulose derivative compositions."

10 An object of the present invention is to provide cellulose derivative compositions of improved water resistance. A further object is to provide cellulose derivative compositions which are substantially permanently flexible, and having improved durability. Other objects will be apparent from the description of the invention hereinafter given.

The above objects are accomplished according to the present invention by the use of esters 20 of organic polycarboxylic acids, at least one acid hydrogen atom of which has been replaced by a normal saturated aliphatic radical containing from 10-15 carbon atoms, inclusive, as a plasticizer for the cellulose derivative.

25 The invention contemplates within its scope the use of esters of any of the organic polycarboxylic acids, whether belonging to the aromatic or aliphatic series. One or more of the carboxylic hydrogen atoms is replaced by a normal saturated 30 aliphatic radical containing from 10-15 carbon atoms corresponding to the following list of alcohols:

|              |                                    |
|--------------|------------------------------------|
| n-decyl      | C <sub>10</sub> H <sub>21</sub> OH |
| n-undecyl    | C <sub>11</sub> H <sub>23</sub> OH |
| lauryl       | C <sub>12</sub> H <sub>25</sub> OH |
| n-tridecyl   | C <sub>13</sub> H <sub>27</sub> OH |
| myristyl     | C <sub>14</sub> H <sub>29</sub> OH |
| n-pentadecyl | C <sub>15</sub> H <sub>31</sub> OH |

40 The esters may contain only one of the above listed alkyl groups and may contain a free carboxylic acid group. Alternatively, an ester containing one normal saturated aliphatic group having 10-15 carbon atoms, may have another 45 carboxylic acid group esterified with any other alcohol. The invention also includes the use of esters of polycarboxylic acids in which more than one acid hydrogen is replaced with a normal saturated aliphatic group having from 10-15 carbon atoms. Accordingly, the invention includes the 50 use of neutral esters of organic polycarboxylic acids in which all of the carboxylic acid groups are esterified, such esters containing one or more of the alkyl groups listed above.

55 The polycarboxylic acids which may be esterified to yield the esters included within the present invention may contain two or more carboxylic acid groups. The following organic acids are named as typical of those which may be used:

orthophthalic, terephthalic, oxalic, succinic, 60 adipic, maleic, fumaric, tartaric, malic, citric, quinolinic, trimesic, pyromellitic, naphthalic, naphthalene tetracarboxylic, tricarballylic, hexahydrophthalic, hydroxy phthalic, uvitic, tetrachlorophthalic, sebacic, itaconic, and pimelic. 65

These esters are preferably made by bringing together the desired alcohols and acids (or where the anhydride of the polycarboxylic acid is available it may be used in lieu of the acid) and then heating the mixture, preferably at temperatures 70 above 100° C. so that the water produced by the esterification will boil off and thus permit the reaction to go to completion. The removal of this water may be assisted by adding to the esterification mixture a carrier liquid, such as benzene 75 or toluene, which will distill out with the water at a temperature below 100° C., in which case the esterification may be carried on at a lower temperature than would otherwise be used. An inert gas, such as carbon dioxide, may be continuously passed through the reacting mixture to accomplish the same purpose, namely, to facilitate the removal of water.

The following examples are given to illustrate typical molding and lacquer cellulose derivative 85 compositions employing the above described esters as plasticizers for the cellulose derivative:

## MOLDING COMPOSITIONS

## Example 1

|                    | Parts |
|--------------------|-------|
| Cellulose nitrate  | 100   |
| Dilauryl phthalate | 35    |

## Example 2

|                     | Parts |
|---------------------|-------|
| Cellulose nitrate   | 100   |
| Dilauryl phthalate  | 20    |
| Tricresyl phosphate | 15    |
|                     | 100   |

## Example 3

|                    | Parts |
|--------------------|-------|
| Cellulose acetate  | 100   |
| Dilauryl phthalate | 30    |

## Example 4

|                    | Parts  |
|--------------------|--------|
| Cellulose acetate  | 100    |
| Dilauryl phthalate | 20     |
| Triacetin          | 15 110 |

## Example 5

|                        |     |       |
|------------------------|-----|-------|
| Cellulose nitrate      | 100 | Parts |
| Lauryl butyl phthalate | 35  |       |

5

## Example 6

|                            |     |       |
|----------------------------|-----|-------|
| Cellulose nitrate          | 100 | Parts |
| Cyclohexyl decyl phthalate | 35  |       |

10

## LACQUER COMPOSITIONS

## Example 7

|                      |       |       |
|----------------------|-------|-------|
| Cellulose nitrate    | 12    | Parts |
| Damar                | 3     |       |
| Lauryl butyl adipate | 4     |       |
| Castor oil           | 2.6   |       |
| Solvent              | 166.5 |       |

20

## Example 8

|                    |    |       |
|--------------------|----|-------|
| Benzyl cellulose   | 4  | Parts |
| Dilauryl succinate | 1  |       |
| Hexyl caproate     | 1  |       |
| Solvent            | 24 |       |

25

## Example 9

|                  |    |       |
|------------------|----|-------|
| Benzyl cellulose | 4  | Parts |
| Damar            | 1  |       |
| Didecyl adipate  | 1  |       |
| Solvent          | 24 |       |

30

## Example 10

|                   |       |       |
|-------------------|-------|-------|
| Cellulose nitrate | 12.0  | Parts |
| Damar             | 3.0   |       |
| Dilauryl adipate  | 4.0   |       |
| Pigment           | 16.3  |       |
| Castor oil        | 2.6   |       |
| Solvent           | 161.6 |       |

40

## Example 11

|                   |       |       |
|-------------------|-------|-------|
| Cellulose nitrate | 12    | Parts |
| Damar             | 3     |       |
| Didecyl phthalate | 4     |       |
| Castor oil        | 2.6   |       |
| Solvent           | 166.5 |       |

In the above examples, showing lacquer compositions, any suitable solvent, such as a mixture of alcohols and esters and hydrocarbons, may be used, as will be understood by those skilled in the art. Solvents may also be used with the molding compositions, if desired. As will also be obvious to those skilled in the art, various gums, natural or synthetic resins, such as polyhydric alcohol-polybasic acid or phenol-formaldehyde resins, pigments, and the like, may be included in these compositions.

Not only dicarboxylic acid esters may be used, as shown in the above compositions, but also tricarboxylic, or higher polycarboxylic acid esters may be used, such as trilauryl citrate. The cellulose derivative compositions containing the esters described above may be used either as lacquers or as molding compositions, as shown in the above examples, or as dopes for use in the preparation of coated fabrics. In the case of the lacquers and the dopes, they may be applied by spraying, brushing, flowing, spreading under a doctor knife, or by other suitable methods of application. When used as molding compositions they can be molded according to the known methods of the plastic art. They also can be pressed into cakes and sheeted to form comparatively thin films which find use as strengthening layers

for safety glass and in other applications where materials of this sort are regularly used.

The cellulose derivative compositions, which may include esters or ethers, are characterized by the fact that they are exceptionally resistant to water, since the plasticizers used in these compositions are all esters of higher aliphatic alcohols having substantial water resistance. The compositions are exceptionally durable and substantially permanently flexible, due to the use of the herein described esters as plasticizers. These esters have higher molecular weights than the commonly used plasticizers and, consequently, have higher boiling points and lower vapor pressures, properties which insure substantially permanent retention of the plasticizer in the cellulose derivative composition, and hence a flexible and durable product. The esters are satisfactorily compatible with cellulose derivatives and give compositions of exceptionally favorable properties.

As many apparently widely different embodiments of this invention may be made without departing from the spirit and scope thereof, it is to be understood that we do not limit ourselves to the specific embodiments thereof except as defined in the appended claims.

We claim:

1. A composition of matter comprising a cellulose derivative and an ester of an organic polycarboxylic acid, at least one acid hydrogen atom of which has been replaced by the radical of a normal primary monohydric aliphatic alcohol containing from 10-15 carbon atoms, inclusive.

2. A composition of matter comprising a cellulose derivative and a neutral ester of an organic polycarboxylic acid, at least one acid hydrogen atom of which has been replaced by the radical of a normal primary monohydric aliphatic alcohol containing from 10-15 carbon atoms, inclusive.

3. A composition of matter comprising a cellulose derivative and an ester of an organic polycarboxylic acid, each of the acid hydrogen atoms of which have been replaced by the radical of a normal primary monohydric aliphatic alcohol containing from 10-15 carbon atoms, inclusive.

4. A composition of matter comprising a cellulose derivative and an ester of an organic dicarboxylic acid, at least one acid hydrogen atom of which has been replaced by the radical of a normal primary monohydric aliphatic alcohol containing from 10-15 carbon atoms, inclusive.

5. A composition of matter comprising a cellulose derivative and a neutral ester of an organic dicarboxylic acid, at least one acid hydrogen atom of which has been replaced by the radical of a normal primary monohydric aliphatic alcohol containing from 10-15 carbon atoms, inclusive.

6. A composition of matter comprising a cellulose derivative and an ester of an organic dicarboxylic acid, each of the acid hydrogen atoms of which have been replaced by the radical of a normal primary monohydric aliphatic alcohol containing from 10-15 carbon atoms, inclusive.

7. A composition of matter comprising a cellulose derivative and an ester of a phthalic acid, at least one acid hydrogen atom of which has been replaced by the radical of a normal primary monohydric aliphatic alcohol containing from 10-15 carbon atoms, inclusive.

8. A composition of matter comprising a cellulose derivative and a neutral ester of a phthalic acid, at least one acid hydrogen atom of which has been replaced by the radical of a normal primary

|                                                                                                                                                                                                                                                                          |                                                                                                                                                                                                                                                                                                                                      |     |
|--------------------------------------------------------------------------------------------------------------------------------------------------------------------------------------------------------------------------------------------------------------------------|--------------------------------------------------------------------------------------------------------------------------------------------------------------------------------------------------------------------------------------------------------------------------------------------------------------------------------------|-----|
| monohydric aliphatic alcohol containing from 10-15 carbon atoms, inclusive.                                                                                                                                                                                              | lulose derivative and di-normal primary decyl adipate.                                                                                                                                                                                                                                                                               |     |
| 9. A composition of matter comprising a cellulose derivative and an ester of a phthalic acid, each of the acid hydrogen atoms of which have been replaced by the radical of a normal primary monohydric aliphatic alcohol containing from 10-15 carbon atoms, inclusive. | 14. A composition of matter comprising a cellulose derivative and normal primary decyl cyclohexyl phthalate.                                                                                                                                                                                                                         | 80  |
| 10. A composition of matter comprising a cellulose derivative and a normal primary decyl phthalate.                                                                                                                                                                      | 15. A composition of matter comprising a cellulose derivative and an ester of an organic dicarboxylic acid of the group consisting of phthalic and adipic acids, at least one acid hydrogen of which has been replaced by a normal primary decyl radical.                                                                            | 85  |
| 11. A composition of matter comprising a cellulose derivative and di-normal primary decyl phthalate.                                                                                                                                                                     | 16. A composition of matter comprising a cellulose derivative and an ester of an organic dicarboxylic acid of the group consisting of phthalic and adipic acids, at least one acid hydrogen of which has been replaced by the radical of a normal primary monohydric alcohol containing from ten to fifteen carbon atoms, inclusive. | 90  |
| 12. A composition of matter comprising a cellulose derivative and an ester of adipic acid, at least one acid hydrogen atom of which has been replaced by the radical of a normal primary monohydric aliphatic alcohol containing from 10-15 carbon atoms, inclusive.     | GEORGE DE WITT GRAVES. 95<br>WALTER EASTBY LAWSON.                                                                                                                                                                                                                                                                                   |     |
| 13. A composition of matter comprising a cel-                                                                                                                                                                                                                            |                                                                                                                                                                                                                                                                                                                                      |     |
| 25                                                                                                                                                                                                                                                                       |                                                                                                                                                                                                                                                                                                                                      | 100 |
| 30                                                                                                                                                                                                                                                                       |                                                                                                                                                                                                                                                                                                                                      | 105 |
| 35                                                                                                                                                                                                                                                                       |                                                                                                                                                                                                                                                                                                                                      | 110 |
| 40                                                                                                                                                                                                                                                                       |                                                                                                                                                                                                                                                                                                                                      | 115 |
| 45                                                                                                                                                                                                                                                                       |                                                                                                                                                                                                                                                                                                                                      | 120 |
| 50                                                                                                                                                                                                                                                                       |                                                                                                                                                                                                                                                                                                                                      | 125 |
| 55                                                                                                                                                                                                                                                                       |                                                                                                                                                                                                                                                                                                                                      | 130 |
| 60                                                                                                                                                                                                                                                                       |                                                                                                                                                                                                                                                                                                                                      | 135 |
| 65                                                                                                                                                                                                                                                                       |                                                                                                                                                                                                                                                                                                                                      | 140 |
| 70                                                                                                                                                                                                                                                                       |                                                                                                                                                                                                                                                                                                                                      | 145 |
| 75                                                                                                                                                                                                                                                                       |                                                                                                                                                                                                                                                                                                                                      | 150 |